

## UNITED STATES PATENT OFFICE

MAX KEVELSON, OF NEW YORK, N. Y.

## IMPREGNATION OF ELECTRICAL CONDENSERS

No Drawing.

Application filed May 24, 1929. Serial No. 365,783.

My present invention relates generally to electrical condensers and has particular reference to the impregnation of condenser bodies of the so-called "paper dielectric" type.

Condensers of the character to which my invention has particular reference are generally formed by interwinding layers of conductive and non-conductive material. For example, foil might be interwound with strips of paper or similar impregnable and non-conductive material, the wound condenser body being subsequently compressed into a substantially flattened shape, suitably treated for purposes of drying, and impregnated with a dielectric material.

It is a general object of my present invention to provide an electrical condenser body of the foregoing character wherein an improved impregnating material, in the form of a novel composition of matter, is employed.

It is well known that the impregnating medium is of paramount importance in producing a condenser of high efficiency. An ideal condenser body would be totally devoid of any non-conducting material such as paper, the strips of paper or the like being employed simply for practical reasons in facilitating the proper interwinding and mutual insulation of the conductive strips. Accordingly, it is highly desirable to impregnate the condenser body with a material having a high dielectric constant, which is not too expensive, and which lends itself readily to thorough impregnation throughout the entire condenser body and particularly throughout the fibers of the paper or similar insulating strips.

Besides a high dielectric constant, it is necessary that the impregnating material be one which does not too easily permit the passage therethrough of leakage current. The so-called "breakdown" of condensers of the character to which this invention relates is a phenomenon the causes of which are not fully understood. Thus, condensers may fail in certain cases because of what is believed to be an excessive void formation and internal ionization. In other cases, failures

may be due to physical leakage, allowing entrance of air or moisture. In many instances, breakdown has been found to be the ultimate result of some sort of heat phenomena, the unwinding of a broken-down condenser often disclosing holes with burnt or charred edges. Besides having a high dielectric constant, it is therefore desirable that the impregnating material be one which prevents, to the maximum possible degree, premature breakdown, whatever the exact cause may be.

It is a more particular object of the present invention to provide an impregnated condenser of the foregoing character wherein the impregnating medium is such that the likelihood of breakdown, even at relatively high voltages, has been minimized, and wherein the life of the condenser has thereby been considerably increased.

The employment of oil has comparatively recently found favor as an impregnating medium for condensers of the type herein referred to. It has advantageous and desirable characteristics of long life, probably due to the fact that its sustained liquid condition facilitates the dissipation of heat induced by minute leakage currents. Furthermore, its liquid condition serves to reduce the formation of undesirable voids. And not only is its own conductivity for leakage currents in many cases less than that of the wax customarily employed for impregnation, but it does not absorb moisture to any appreciable degree, and its leakage conductivity is thereby not increased with time as is frequently the case with wax, as, for example, paraffine.

One of the features of my invention resides in the employment, as an impregnating material, of an oily substance or composition of matter whereby the foregoing advantageous characteristics are made use of. One of the disadvantages of oil lies in the fact that its normally liquid condition renders it less cohesive than a relatively solid material such as wax, and as a result, it is not as efficacious in firmly holding the layers forming the condenser body in close superposition. Accordingly, although its dielectric strength may be substantially the same as that of wax or the

like, it has proven comparatively expensive as compared with wax.

An important object of my present invention is to provide an improved composition of matter for the impregnation of condenser bodies wherein the advantageous characteristics of oil are maintained while the dielectric constant has been sufficiently increased to render the employment thereof highly advantageous from all standpoints, including that of manufacturing cost.

Briefly, my invention resides in the employment of at least two different oils capable of mutual intimate intermixture thereof, 15 suitably inexpensive and available on the market so as to render the commercial employment thereof feasible, and imbued with characteristics which complement each other in the production of a highly efficient and 20 relatively inexpensive condenser of great strength and long life.

From one aspect, the invention resides in the employment of mineral oil in combination with a second and different type of oil which 35 complements the mineral oil and produces a resultant composite oily composition of matter of highly desirable characteristics so far as the impregnation of condensers is concerned. More specifically, I employ a second oil which has a relatively high dielectric constant, which would be wholly unsatisfactory for use by itself, and which blends nevertheless with mineral oil in such a manner that the ultimate intermixture embodies all the 35 desirable characteristics of mineral oil, and in addition, a relatively high dielectric strength and constant.

More specifically, I have found that castor oil is suitable for my present purposes. All 40 vegetable oils seem to have a high leakage conductivity and are therefore unusable by themselves for electrical purposes. Castor oil is no exception in this respect since it has a considerable affinity for moisture; but it assumes importance from the standpoint of my 45 present aims and objects by virtue of the fact that it has a very high dielectric constant, viz., approximately 4 as distinguished from the average dielectric constant 2 of mineral oil.

Although mineral oil and castor oil will not ordinarily blend, it is possible nevertheless to cause an intimate intermixture thereof in a number of ways. For example, by mixing the two and raising the temperature to several hundred degrees centigrade under pressure, a suitable blending may be effected. Apparently, the castor oil polymerizes in such a manner that the two oils will mix in all proportions and will remain in intimate blended relationship even after the temperature has subsequently been reduced to normal condition.

It might appear that the advantage gained 55 by the high dielectric constant of the castor

oil might be offset by its correspondingly high leakage current conductivity. I have found, however, that the normally high leakage current conductivity of the castor oil seems to disappear entirely when a blending or intimate intermixture of the foregoing character has been effected. As a matter of fact, the resultant oily composition of matter acts in many ways as a pure mineral oil having no less resistance to the passage of leakage currents than that of pure mineral oil. On the other hand, however, I have found that the oily compound of these two oils has a dielectric constant considerably higher than that of the mineral oil by itself. 80 For example, depending entirely upon the proportions in which the two oils are intermixed, the resultant composition of matter may be caused to embody a dielectric constant of anywhere from 2 to 4. 85

In carrying the invention into practical effect, the condenser bodies are formed or wound in the customary manner and vacuum-treated and dried in accordance with well-known practice. They are then impregnated 90 with the composite oil resulting from an intimate intermixture or blending of mineral and castor oils. I have found an intermixture in the proportion of 60-70% of castor oil and 40-30% of mineral oil to be highly 95 satisfactory, the product having a dielectric constant of approximately 3.5 and a leakage current conductivity no greater than that of ordinary mineral oil.

Stated otherwise, the mixture produced in 100 accordance with my invention is one wherein the advantageous characteristics of the mineral oil have been retained, wherein the advantageous high dielectric constant of castor oil has materially contributed to an increased 105 dielectric constant of the mixture, and wherein the objectionable leakage current conductivity initially present in the pure castor oil has apparently vanished, at least so far as an increase of leakage current conductivity of 110 the resultant intermixture is concerned. The advantages of such an impregnating medium need hardly be elaborated upon.

By the term "mineral oil", as the same is employed herein and in the appended claims, 115 it will be understood that I refer to any natural oil of the petroleum series, such as paraffine-base oil, naphthene-base oil, olefine-base oil, or combinations of these oils. Any oil of this general class may be employed in 120 carrying out my present invention.

I do not mean to limit myself to any specific proportions of the two ingredients nor to any particular manner of blending the same, except insofar as either of these factors 125 is essential to produce the advantageous result desired.

In general, it will be obvious that changes in the details herein described for the purpose of explaining the nature of my inven- 130

tion may be made by those skilled in the art without departing from the spirit and scope of the invention as expressed in the appended claims. It is therefore intended that these details be interpreted as illustrative and not in a limiting sense.

Having thus described my invention, what I claim as new and desire to secure by Letters Patent is—

10 1. As a new article of manufacture, an electrical condenser in which the dielectric employed therein comprises a mineral oil and castor oil blended substantially as described.

15 2. As a new article of manufacture, an impregnated electrical condenser body in which the dielectric impregnating medium comprises an intimate intermixture of two oils, one of which has a relatively low dielectric constant and a relatively high dielectric resistance, the other of which has a relatively high dielectric constant and a relatively low dielectric resistance, whereby said body is impregnated with an oily medium embodying the advantageous electrical qualities of both oils.

20 3. An electrical condenser body comprising alternate layers of conductive and non-conductive material and impregnated with an oily dielectric medium comprising an intimate intermixture of castor oil and mineral oil in the proportion of approximately 60-70% of castor oil to 40-30% of mineral oil.

25 4. As a new composition of matter for the impregnation of electrical condenser bodies, an intimate intermixture of castor oil and mineral oil, said oils being blended as the result of heating thereof under pressure.

30 40 In witness whereof I have signed this specification this 20th day of May, 1929.

MAX KEVELSON.

45

50

55

60

65